# EUROPEAN PATENT SPECIFICATION

(11) **EP 2 125 310 B1**
(45) Date of publication and mention of the grant of the patent: **26.10.2011**
(21) Application number: 08724036.2
(22) Date of filing: 20.03.2008
(51) Int. Cl.: B27K 7/00

(54) **PROCESS OF CORK PRE-EXPANSION BY SUBMISSION TO MICROWAVE RADIATION**
VERFAHREN ZUR VOREXPANSION VON KORK DURCH BESTRAHLUNG MIT MIKROWELLEN
PROCESSUS DE PRE-EXPANSION DU LIEGE PAR SOUMISSION A UN RAYONNEMENT A MICRO-ONDES

(30) Priority: 21.03.2007 PT 10369707
(43) Date of publication of application: 02.12.2009
(73) Proprietor: Amorim Cork Composites, S.a., 4536-902 Mozelos Vfr (PT); Amorim Isolamentos, S.a., 4535-173 Mozelos Vfr (PT)
(72) Inventor: PEREIRA, Helena Margarida Nunes, P-1170-179 Lisboa (PT); REIS, Rui Luis Gonçalves dos, P-4250-242 Porto (PT); MARTINS, Susana Pinto Araújo da Silva Estima, P-4470-193 Maia (PT); MARQUES, Antonio Jorge Velez, 2665-314 Milharado (PT)
(74) Representative: Alves Moreira, Pedro
(86) International application number: PCT/PT2008/000012
(87) International publication number: WO 2008/115086

(56) References cited:
- WO-A-99/37334
- WO-A-2006/021225
- SILVA S P ; SABINO M A ; FERNANDAS E M ; CORRELO V M ; BOESEL L F ; REIS R L: "Cork: Properties, capabilities and applications" INTERNATIONAL MATERIALS REVIEWS, vol. 50, no. 6, December 2005 (2005-12), pages 345-365, XP002482488

## Description

### FIELD OF THE INVENTION

This invention relates to a process, and to the resulting material, that allows the volumetric expansion of cork without using substances foreign to the cork system. More precisely, it relates to a process that consists in submitting cork to microwave radiation, obtaining a more bulky material and consequently increasing its yield and reducing its specific weight.

### BACKGROUND OF THE INVENTION

In general, to promote the expansion of cork or cork derivatives, water or water vapour is used at different stages of its workup process. The applicant has already developed an improved method of expansion by water vapour.

The expansion of cork from values of 70% to 220%, shown in the Portuguese Patent PT101215, is performed by the use of organic solvents in autoclave.

Another way of achieving expansion of cork or of different cork derivatives is the processing by microwaves.

Microwave radiations can be used on cork as a way of cork sterilization or decontamination, as described in the international patent no. WO9937334. On the other hand, the German patent no. DE019523 refers in addition to the possibility of sterilization, the elimination of 2,4,6-trichloroanisol (known as TCA). The elimination of parasites, insects, bacteria or fungi by the action of microwave radiation is disclosed in the international patent no. WO2006021231. The purpose in both patents is to clean the cork, so it is not in the scope of the present application.

The European patent no. EP1677386 claims that wood, a material different from cork but also lignocellulosic, can be submitted to microwave radiations in order to destroy insects, parasites or their larvae. Moreover, the international patent no. WO03002923, describes the use of microwave radiation for fast wood drying, increasing additionally its permeability. In that case, the use of microwaves radiation is applied for wood cleaning, so its scope is not within the present application.

Microwave radiations are also used to cure polymers such as latex, as described in the Spanish patent no. ES2019514, or to cure resins for the production of wood derivatives, as described in the international patent no. WO9823132. Again, the scope of these inventions is different from the present application.

Concerning the cork material obtained by the process herein, it is also important to emphasize the volumetric increase effect observed on the specific weight.

Microscopically, cork can be described as a homogeneous tissue of thin cells, without space between them, and an alveolar structure similar to a honeycomb. The cork cells show diverse shapes depending if observed on the radial direction (Figure 1) or in a perpendicular direction to radial, i.e., axial or tangential (Figure 2).

The closed structure of cork cells and the presence of air inside determine the low specific weight of cork, as well as some of its mechanical properties. The specific weight of cork might however show a significant variability, between 120kg.m⁻³ and 240kg.m⁻³, as described by M. Fortes in the Boletim do Instituto dos Produtos Florestais - Cortiça, 1988, pages 65-68. This variability is essentially related to the cell dimensions (height and thickness of wall), corrugation of cell walls and quantity of lenticels. It should be emphasized that lower values of cork specific weight represent higher economical value.

Given the mathematical relation between volume and specific weight (inversely proportional), the volumetric increase (in the three spatial directions) observed in samples submitted to microwave treatment, and with maintenance of the initial mass, represents the gain achieved by this process in the cork specific weight.

### BRIEF DESCRIPTION OF THE DRAWINGS

The invention description is supported by:
- Figure 1 and Figure 2, which show a scheme of the radial and axial/tangential directions of cork cells, respectively.
- Figure 3, which shows a table with the operational conditions and the expansion results of cork samples by submission to microwave radiation, after humidification by water immersion.
- Figure 4, which shows a table with the operational conditions and the expansion results of cork samples by submission to microwave radiation, after humidification in autoclave.

### DETAILED DESCRIPTION OF THE INVENTION

The present application describes a process capable of promoting cork expansion without using external substances to the cork system. Subsequently, the produced cork might be submitted to standard cork industrial processes.

This process can be used in continuous or non-continuous mode and has three stages, the first stage being the dosing of the material, followed by the expansion stage, and finally the discharge stage or preferably cooling and discharge.

In the case of a continuous process for cork expansion by submission to microwave radiation, the dosing stage intends to feed continuously and over time the expansion zone and can be done using a feeding endless screw or a conveyor. The expansion stage should ensure the contact of the product to the action of the microwave radiation by a conveyor or dielectric containers such as for example, fibber glass, wood, plywood, among others. The radiation power should range between 200 watt and 1000 watt, preferably between 400 watt and 800 watt. The exposure time to the microwave radiation should be between 10 seconds and 5 minutes, preferably between 15 seconds and 2 minutes or even more preferably between 15 seconds and 50 seconds. The collecting stage could be performed using an endless screw that might have a sealant "lock", a manual or electropneumatic plate valve or a conveyor. During the expansion, process by submission to microwave radiation the presence of moisture is crucial for the expansion to occur. The samples should have a humidity higher than 5%, which can be achieved by immersion in water at temperature ranging between 25 °C and 100 °C or by autoclave at temperatures between 100 °C and 150 °C.

In the case of a non-continuous process for cork expansion by submission to microwave radiation, the dosing stage aims to feed the microwave chamber and can be performed using a feeding endless screw that may have a dosing sealant "lock" or a manual or electropneumatic plate valve or a conveyor. The cork expansion stage will occur inside a closed chamber made of a dielectric material such as, for example, glass fibber, wood, plywood, among others. The radiation power should range between 200 watt and 1000 watt, preferably between 400 watt and 800 watt. The exposure time to the microwave radiation should be between 10 seconds and 5 minutes, preferably between 15 seconds and 2 minutes or even more preferably between 15 seconds and 50 seconds. The expansion stage by submission to microwave radiation can be performed in one or more cycles. When performed on several cycles, this number might range between 2 and 15, preferably between 2 and 5. The time period of each of these cycles could range between 2 seconds and 15 minutes, preferably between 2 seconds and 1 minute. The product collecting stage in the non-continuous process for cork expansion by submission to microwave radiation can be performed using an endless screw that may have a sealant "lock" or a manual or electropneumatic plate valve or a conveyor. During the expansion, process by submission to microwave radiation the presence of moisture is crucial for the expansion to occur.

### Product resulting from the pre-expansion process

The present application seeks to demonstrate the increase of the cork dimensions and consequently the decrease of its specific weight after submission to microwave radiation.

The cork can be submitted to this pre-expansion process independently of its shape, origin, quality or pre-treatments already performed, namely, falca cork, virgin or reproduction cork, cork planks, cork residues (resulting from stopper production or cork plank transformation), grinded cork, granulated cork or cork powder, any of them boiled or not boiled.

The increase on cork dimensions, after being submitted to microwave radiations with controlled moisture, has two effects: promotes a yield increase of the material, i.e., less material used for the same application; and promotes an increase of the material quality, due to the reduction in specific weight. These two aspects represent commercial benefit.

### RESULTS

The submission of cork to a pre-expansion process by microwave radiation for time periods between 5 seconds and 5 minutes, results in expansion of the initial material between 40% and 85%. During this process, no expansion in samples with less than 5% of humidity was observed.

The cork material such as falca cork, virgin or reproduction cork, cork planks, cork residues (resulting from stopper production or cork plank transformation), grinded cork, granulated cork or cork powder, any of them boiled or not boiled, shows an increase on its dimensions between 40% and 85%, when submitted to a pre-expansion process by submission to microwave radiation such as above described. This fact implies the reduction of its specific weight. It should be emphasized that in addition to the increase on the material yield (higher volume of cork after the treatment), the cork with lower specific weight presents higher economical value.

Application examples of the pre-expansion process and respective results are presented herein below:

### - Example 1: Cork expansion by submission to microwave radiation.

Cubic shaped cork samples were submitted to microwave radiation with 550 watt power. One group of samples was exposed for 25 seconds whereas another group was exposed to five cycles of 5 seconds each. The observed expansions were, respectively, 48% and 46%, emphasizing the importance of the exposure time and not the operation mode (continuous or several cycles).

### - Example 2: Cork expansion with different humidity by submission to microwave radiation.

Cubic shaped cork samples were submitted to microwave radiation with 550 watt power. A group of samples with 1.4% of humidity presented, after treatment, a volumetric expansion of 0.6%. Another group of samples with 7-10% of humidity presented, after treatment, a volumetric expansion of 40-45%. This example emphasizes the importance of moisture in the samples for the expansion to occur.

### - Example 3: Cork expansion by submission to microwave radiation after humidification by water immersion.

Cubic shaped cork samples were submitted to microwave radiation, after immersion in water at different temperatures and for different time periods. The results of the expansion and the detailed conditions are presented in Figure 3. Besides showing the microwave radiation effect on the volumetric increase of cork samples, expansion between 40% and 65%, these results allow to conclude that humidification by immersion in water is a possible method to be used, the immersion water temperature having a positive effect on the cork volumetric expansion.

### - Example 4: Cork expansion by submission to microwave radiation after autoclave humidification

Samples of virgin and amadia cork, with cubic shape, were submitted to microwave radiation, after autoclave humidification for different time periods. The results of the expansion and the detailed conditions are presented in the table of Figure 4. In addition of showing the effect of microwave radiation in cork volumetric increase, these results of expansion between 40% and 85%, make possible to conclude that the humidification in autoclave is a possible method to adopt, the virgin cork showing higher values of expansion when compared with amadia cork.

The process of cork pre-expansion by submission to microwave radiation and resulting products described above can be subjected to many modifications and variations performed by a person skilled in the art in order to adjust to specific requirements, which are within the scope of the present invention, as defined by the following claims.

## Claims

1. Process for pre-expansion of cork by submission to microwave radiation **characterised in that** it comprises the following stages:
a) dosing, comprising cork feeding with a humidity higher than 5% to the expansion zone,
b) expansion by the action of microwave radiation, and
c) discharge of the expanded cork.

2. Process for pre-expansion of cork according to claim 1 **characterised in that**, in the expansion stage a microwave radiation of 200 to 1000 Watt power is applied for a period of about 10 seconds to 5 minutes.

3. Process for pre-expansion of cork according to claim 1 **characterised in that**, in the expansion stage a microwave radiation of 400 to 800 Watt power is applied for a period of about 15 seconds to 2 minutes.

4. Process for pre-expansion of cork according to claim 1 **characterised in that**, in the expansion stage 2 to 15 cycles of microwave radiation are applied, each one with a time period of 2 seconds to 15 minutes.

5. Process for pre-expansion of cork according to claim 1, **characterised in that** it is performed in continuous or non-continuous mode.

6. Process for pre-expansion of cork according to claim 1 **characterised in that**, the discharge stage is preceded by cooling of the expanded cork.

7. Process for pre-expansion of cork according to claim 1 **characterised in that**, the dosing stage is preceded by a cork humidification step by water immersion at temperatures between 25 and 100 °C or in autoclave at temperatures between 100 °C e 150 °C.

8. Process for pre-expansion of cork according to claim 1, **characterised in that** the cork is selected from the group comprising falca cork, virgin or reproduction cork, cork planks, cork residues resulting from stopper production or from cork plank transformation, grinded cork, granulated cork or cork powder.

## Patentansprüche

1. Verfahren zur Vorexpansion von Kork durch Bestrahlen mit Mikrowellen, **dadurch gekennzeichnet, dass** dieses die folgenden Phasen umfasst:
a) Dosieren, umfassend das Zuführen von Kork mit einer Feuchte über 5% zu dem Expansionsbereich,
b) Expansion durch das Einwirken von Mikrowellenstrahlung, und
c) Austragen des expandierten Korks.

2. Verfahren zur Vorexpansion von Kork nach Anspruch 1, **dadurch gekennzeichnet, dass** in der Expansionsphase Mikrowellenstrahlung mit 200 bis 1000 Watt Leistung während eines Zeitraums von etwa 10 Sekunden bis 5 Minuten angewandt wird.

3. Verfahren zur Vorexpansion von Kork nach Anspruch 1, **dadurch gekennzeichnet, dass** in der Expansionsphase Mikrowellenstrahlung mit 400 bis 800 Watt Leistung während eines Zeitraums von etwa 15 Sekunden bis 2 Minuten angewandt wird.

4. Verfahren zur Vorexpansion von Kork nach Anspruch 1, **dadurch gekennzeichnet, dass** in der Expansionsphase 2 bis 15 Zyklen Mikrowellenstrahlung angewandt werden, jeder über einen Zeitraum von 2 Sekunden bis 15 Minuten.

5. Verfahren zur Vorexpansion von Kork nach Anspruch 1, **dadurch gekennzeichnet, dass** dieses im kontinuierlichen oder diskontinuierlichen Betrieb durchgeführt wird.

6. Verfahren zur Vorexpansion von Kork nach Anspruch 1, **dadurch gekennzeichnet, dass** der Austragsphase das Kühlen des expandierten Korks vorausgeht.

7. Verfahren zur Vorexpansion von Kork nach Anspruch 1, **dadurch gekennzeichnet, dass** der Dosierphase ein Korkbefeuchtungsschritt durch Eintauchen in Wasser bei Temperaturen zwischen 25 und 100°C oder im Autoklaven bei Temperaturen zwischen 100°C und 150°C vorausgeht.

8. Verfahren zur Vorexpansion von Kork nach Anspruch 1, **dadurch gekennzeichnet, dass** der Kork aus der Gruppe umfassend Falca-Kork, Primär- oder Reproduktionskork, Korkplanken, Korkreste aus der Korkenstöpselherstellung oder Korkplankenverarbeitung, Korkmehl, Korkgranulat oder Korkpuder ausgewählt wird.

## Revendications

1. Procédé de pré-expansion du liège par soumission à un rayonnement à micro-ondes, **caractérisé en ce qu'**il comprend les étapes suivantes:
a) le dosage, comprenant la conduite du liège à la zone d'expansion avec une humidité supérieure à 5 %;
b) l'expansion par l'action d'un rayonnement à micro-ondes; et
c) la décharge du liège expansé.

2. Procédé de pré-expansion du liège selon la revendication 1, **caractérisé en ce que**, lors de l'étape d'expansion, un rayonnement à micro-ondes d'une puissance de 200 à 1000 watts est appliqué pendant une période d'environ 10 secondes à 5 minutes.

3. Procédé de pré-expansion du liège selon la revendication 1, **caractérisé en ce que**, lors de l'étape d'expansion, un rayonnement à micro-ondes d'une puissance de 400 à 800 watts est appliqué pendant une période d'environ 15 secondes à 2 minutes.

4. Procédé de pré-expansion du liège selon la revendication 1, **caractérisé en ce que**, lors de l'étape d'expansion, 2 à 15 cycles de rayonnement à micro-ondes sont appliqués, chacun pendant une période de temps d'environ 2 secondes à 15 minutes.

5. Procédé de pré-expansion du liège selon la revendication 1, **caractérisé en ce qu'**il est exécuté en mode continu ou discontinu.

6. Procédé de pré-expansion du liège selon la revendication 1, **caractérisé en ce que** l'étape de décharge est précédée par un refroidissement du liège expansé.

7. Procédé de pré-expansion du liège selon la revendication 1, **caractérisé en que** l'étape de dosage est précédée par une étape d'humidification du liège par immersion dans l'eau à des températures comprises entre 25°C et 100°C, ou dans un autoclave à des températures comprises entre 100°C et 150°C.

8. Procédé de pré-expansion du liège selon la revendication 1, **caractérisé en ce que** le liège est sélectionné dans le groupe comprenant le liège falca, le liège mâle ou de reproduction, des planches de liège, des résidus de liège résultant d'une production de bouchons ou d'une transformation de planches de liège, du liège broyé, du liège granulé ou de la poudre de liège.
